

## UNITED STATES PATENT OFFICE

REED P. ROSE, OF JACKSON HEIGHTS, NEW YORK, ASSIGNOR TO GENERAL RUBBER COMPANY, OF NEW YORK, N. Y., A CORPORATION OF NEW JERSEY

## MANUFACTURE OF SHEET MATERIAL

No Drawing.

Application filed December 2, 1928. Serial No. 152,313.

This invention relates to improvements in the manufacture of fibrous sheet material and its primary object is the manufacture of such material containing dispersed rubber and bituminous material. Such products are of particular importance in the art for the reason that they possess a high degree of pliability, great resistance to tear, are plastic and moldable when heated, capable of retaining the shapes or impressions imparted to them while heated, and may be subjected to considerable stretch without tear.

The invention comprises beating paper-making pulp, mixing dispersions of rubber and of bituminous materials with the beaten pulp, coagulating the rubber and bitumen upon the beaten fibres, and subsequently forming the product into sheets or slabs according to the customary methods of manufacture.

The bituminous dispersions may be prepared in any desired manner, as for example by dispersing an asphalt in a non-solvent thereof, preferably water, in the presence of a protective colloid, using any of the machinery or apparatus customarily employed in the manufacture of emulsions, suspensions or dispersions. The invention is not limited to any particular method of manufacturing the dispersions above mentioned, but I prefer that the bituminous material shall be dispersed with a protective agent such as a soap, for example rosin soap, as I believe that the bituminous particles are more firmly attached to the fibres when such a protective agent is used than is the case when colloidal clays are used as the protective agent.

As one illustration of a method of carrying out the invention, a paper making fibre is beaten in water in the usual way customary in the manufacture of paper. When the beating operation has been carried to a sufficient degree for the preparation of the desired sheet, the beater roll is raised and a water dispersion of rubber (preferably latex) and a water dispersion of bituminous material are added to the beater in any desired percentages while the beater roll is

continued in operation, thus operating to bring about a uniform distribution of the paper pulp, rubber and asphalt dispersions. After a uniform distribution is obtained, the rubber and asphalt contents of the beater are precipitated or coagulated upon the paper fibres or pulp by a coagulating process which preferably consists of adding a solution of aluminum sulphate sufficient to neutralize the alkalinity of the beater contents and preferably sufficient to render the contents slightly acid. The coagulating solution is preferably of a 3-5% concentration and while it is being added to the beater the roll is preferably continued in operation to produce a thorough mixing of the beater contents and to obtain such a distribution that the coagulation will go on uniformly throughout the whole mass without being localized so that it will be easily apparent when complete coagulation or deposition of the rubber and asphalt on the beaten fibres has taken place because at that point the water content of the beater will change from a cloudy mass to a condition in which the pulp and adhering asphalt and rubber can clearly be seen as dispersed in a substantially clear water showing quantitative retention on the fibres of the entire contents of dispersed materials. Of course it is understood that the total amount of rubber and bituminous material compared with the fibre contents of the beater may be varied within wide ranges, but a good practice is to add a total of 20-50% of the rubber and asphalt dispersion compared with the dry weight of the fibre. And of course it is understood that the proportion of bituminous material to the rubber may be varied within wide limits as for example, 5-100% of asphalt, compared with the amount of rubber. In ordinary practice I have found a very useful product to be obtained by the use of equal parts of rubber and asphalt.

The treated fibres may now be passed to the stuff chests and to the paper making machine and further handled in accordance with ordinary paper making practice.

Instead of the foregoing method of intro-

55

60

65

70

75

80

85

90

95

100

ducing the rubber and asphalt dispersions, I may introduce the rubber dispersion first and coagulate and deposit the rubber dispersion on the fibre alone. After the rubber has been deposited by the coagulation process upon the fibre as just described, the contents of the beater are made slightly alkaline with caustic soda, ammonia or other suitable alkali. The asphalt dispersion may now be added and after thorough mixing with the beater contents is deposited by coagulation on the fibre by the addition of a further quantity of coagulating material which is preferably added in sufficient quantity to render the contents of the beater appreciably acid in reaction. Of course the procedure immediately above described may be varied by varying the order of addition of the dispersed materials by adding the asphalt dispersion first and then subsequently adding the rubber dispersion.

Sheets containing rubber and asphalt, when prepared as above described, differ widely from sheets containing rubber and asphalt, but made in different ways. The products of this invention have much more pliability than the asphalt-containing sheets heretofore known. Furthermore, the products of the invention are characterized by much greater initial resistance to tear, as well as a greater actual tear resistance, and by a greater degree of stretch, than is found in latex papers or in asphalt sheet materials. These properties are extremely useful in the arts. The rubber and asphalt are intimately associated with the fibres prior to the sheet forming operation, and the products of the invention are therefore different from other sheet materials containing the same ingredients, but where the ingredients are mechanically held by the sheet, as for example when the materials are introduced after the sheet is formed, or when the dispersed materials are not coagulated.

By way of illustration fibrous sheet materials containing rubber and bitumen, prepared as above described, are very satisfactory for use as backing materials for imitation leather, for example automobile toppings, luggage, upholstery, book covers, etc. Certain characteristic properties of the product of this invention are of extreme usefulness in the above instances. The products are characterized by a high degree of moldability, as demonstrated by the sharpness and permanency of embossed impressions made upon the sheet. Another property is pliability, demonstrated by the ease with which the sheet material may be manipulated for covering the tops and lining the interiors of automobiles, and for general upholstery purposes. The high stretch of the fibrous sheet permits the material to be pulled around and over corners and edges without formation of wrinkles.

Thick sheets of the above described material may be used very satisfactorily for the manufacture of box toes and counters for footwear. The above described properties of moldability, pliability and stretch are valuable assets in the manufacture of these and other shoe parts. In this instance a selection of the type of bitumen may be made so that the resulting product is thermoplastic, can be molded while hot, and after cooling will assume the necessary rigidity required by the footwear industry for box toes and counters. In addition to the above mentioned properties which are characteristic of the materials of this invention, there is a very high initial resistance to tear when attempts are made to tear an edge of the material. This is due to the comparatively high stretch of the product, and this property makes it extremely valuable as a stay material or reinforcing material for shoes.

By carefully selecting the fibre, and beating it so as to obtain a short length and high degree of hydration and then incorporating the rubber and bitumen as above described, thick slabs can be made. These thick products show a high resistance to abrasion and great flexibility, and at the same time the slabs are moldable and capable of holding stitches. These thick slabs may be used as outsoles, midsoles, or inner soles for footwear. One satisfactory way of preparing these heavier products is to run the fibre and dispersed material on a standard wet machine. Similar products may be made by first partially removing the water content of the fibre mixture, for example by draining and pressing, and subsequently molding the partially dried fibre in a plunger mold, or by other suitable means, including hydraulic or mechanical presses.

Paper and fibrous sheet material made according to the present invention are more resistant to water than either latex paper or asphalt papers and sheets. Combinations of beaten fibre, dispersed rubber and bituminous material made by the herein-described methods possess the property of running smoothly on paper-making machinery, and the bituminous material does not stick to the wires, felts or rolls, as has always been the case in the prior manufacture of sheet material containing such material, but prepared in other ways.

On account of the molding properties of this material the pulp after deposition of the rubber and asphalt may be molded into articles without first making the sheet. In this instance it is preferable, although not necessary, to remove all of the water from the pulp before the molding operation.

The invention contemplates the use of rubber in any of its dispersions, natural, synthetic or artificial, or mixtures of any of

these. The rubber itself may comprise the globular rubber particles occurring in natural latex, or it may be an artificial latex comprising dispersed crude rubber, vulcanized rubber, reclaimed rubber separately or in admixture with each other, and may include mixtures of these together with other rubber-like gums, etc. For some purposes it may be desirable to include compounding ingredients with the rubber, such as the mineral fillers, pigments, softening agents, such as oils, fats, waxes, resins, rubber substitutes, vulcanizing materials and accelerators. If natural latex be used as the rubber dispersion, it may be compounded in any desired manner, and may or may not be vulcanized prior to its introduction into the beater. The bituminous dispersion may comprise the natural asphalts, earth waxes or mineral waxes, as well as the other mineral pitches, resins, tars, tar residues, condensation products, etc.

If desired, the asphalt dispersion may likewise be compounded in somewhat the same fashion as the rubber dispersion may be mixed with other ingredients.

In view of the latitude which is permissible in the selection of materials forming the internal phase of the dispersions, the terms "rubber dispersion" and "dispersion of reinforcing material" as used in the appended claims are to be broadly construed as including the materials herein described as well as their equivalents. The term "sheet material" as used in the appended claims is to be construed as generic to any of the fibrous products resulting from paper making methods and machinery, and includes slabs of varying thicknesses and paper.

Having thus described my invention, what I claim and desire to protect by Letters Patent is:

1. Process for making fibrous sheet material which comprises beating paper-making pulp, introducing rubber dispersion and bituminous dispersion into the beaten pulp, coagulating the solid material from both dispersions on the pulp, and recovering the treated pulp.

2. Process for making fibrous sheet material which comprises beating paper-making fibre, separately adding rubber and bituminous material in dispersed form, mixing the dispersions with the fibre, and coagulating the solid material on the fibres, and subsequently forming the treated fibres into sheets.

3. Process for making fibrous sheet material which comprises beating paper-making fibre, adding a rubber dispersion to the beaten pulp, mixing said dispersion with the beaten fibre, adding sufficient coagulant to deposit the dispersion on the fibres, introducing a dispersion of bituminous material

before the rubber dispersion is completely coagulated, and completing the coagulation of both dispersions, and forming into sheets.

4. Process for making sheet material which comprises beating fibre, adding a rubber dispersion to the beaten fibre, mixing said dispersion with the beaten fibre, slowly and continuously coagulating the dispersion on the fibres, introducing a dispersion of bituminous material before the rubber dispersion is completely coagulated, and completing the coagulation of both dispersions, and forming into sheets. 70 75

5. Process for making sheet material which comprises beating paper-making fibres, adding a rubber dispersion to the contents of the beater in the presence of alkali, neutralizing the contents of the beater to deposit the rubber on the fibre, introducing further quantities of alkali into the mixture, adding a dispersion of bituminous material, acidifying the resulting mixture and depositing both rubber and bituminous material on the fibres, and subsequently forming the latter into sheets. 80 85 90

6. Process for making fibre sheets which comprises beating paper-making fibre, adding rubber dispersion thereinto in the presence of an alkali, neutralizing the alkali, mixing to distribute the rubber throughout the fibre, introducing a further quantity of alkali, adding an asphalt emulsion to the beaten pulp, acidifying the mixture to deposit both rubber and asphalt upon the fibres, and subsequently forming the latter 95 100 into sheets.

7. Process for making fibrous sheet material which comprises beating paper-making fibres, introducing dispersed rubber and bituminous material into the beaten fibres, coagulating the rubber and bituminous material on the fibres, and forming the treated fibres into sheets. 105

8. As a new product, fibrous sheet material comprising beaten fibres and rubber and bituminous material, the fibres of said product having the characteristics of having been coated with said rubber and bituminous material by coagulation of said rubber and bituminous material from a water dispersion thereof on said fibres in a pulp suspension of the fibres. 110 115

Signed at New York, county and State of New York, this 26th day of November, 1926.

REED P. ROSE. 120